

Patented Aug. 3, 1926.

1,594,830

## UNITED STATES PATENT OFFICE.

THOMAS T. GRAY, OF ELIZABETH, AND WALTER L. FAUST, OF SUMMIT, NEW JERSEY, AND MALVIN R. MANDELBAUM, OF BROOKLYN, NEW YORK, ASSIGNORS TO WHITLOCK CORDAGE COMPANY, OF JERSEY CITY, NEW JERSEY, A CORPORATION OF NEW JERSEY.

### CORDAGE.

No Drawing. Original application filed August 20, 1925, Serial No. 51,506. Divided and this application filed January 26, 1926. Serial No. 83,951.

Our invention relates to improvements in cordage and particularly to ropes, hawsers, and the like, which are intended to be used where they may be exposed to rain, sea water, and other forms of dampness.

The present application is a division of our pending application Serial Number 51,506, filed August 20, 1925, wherein is described and claimed an impregnating compound for use in manufacturing the cordage of the present invention.

A particular object of our invention is to provide cordage in which the fibers are impregnated with a water-resisting and lubricating compound. A further object is to provide cordage which is practically water-proof, so that despite repeated exposure to dampness or wetting, water will not be permitted to enter the cells of the rope fiber and the rope will accordingly remain strong, flexible and easy to handle.

A further object of our invention is to provide cordage which is permanently lubricated despite exposure to moisture.

The stiffness and difficulty of handling wet rope have heretofore presented great disadvantages and danger in use. When ordinary lubricated rope is exposed to dampness the moisture penetrates into and distends the cells of which the fiber is formed, thereby swelling and shortening and tending to kink the rope and making it stiff and unmanageable and at the same time diminishing the natural water-resistant quality of the fiber and driving out a part of the natural and artificial lubricant as well. As the natural waxes and artificial lubricants are driven out the fibers become brittle and tend to disintegrate so that the life of the rope as well as its strength and serviceability are substantially diminished by such exposure. By our invention we provide a rope the fibers of which are impregnated with a compound which is so water-repellent as to make the rope substantially waterproof and we thereby keep moisture out of the fiber cells and retain the natural and artificial lubricants in the fiber and overcome the difficulties heretofore met and provide a rope which is longer lived and superior to any now known.

Other advantages of our invention will be apparent from the following description and claims.

Broadly our invention consists of rope structure made up of cellular fibers the cells of which are impregnated with a stable semi-solid compound containing water-resisting waxes, the said compound being of such character as to be capable of passing as a whole through the walls of the fiber cells and constituting an efficient lubricant for the cordage. The manner of mixing and applying an appropriate impregnating compound to the cordage fiber is described in our original application Serial Number 51,506 referred to.

The impregnating compound, being of the character stated, penetrates to the interior of the cells of which the rope fibers are made up, taking the place of any natural waxes that have been driven out in the course of preparing and shipping the fiber to the cordage plant and supplementing such natural waxes as remain in the fiber in completely filling the cells with stable, water-resisting, lubricating material. The fiber as a whole is given a stability and smoothness, a resistance to wear and to water that results in a rope that is substantially water-proof and permanently lubricated.

A preferred form of our invention comprises a rope structure the fiber cells of which are impregnated and coated with a compound containing waterproofing waxes such as paraffin and Japan wax dissolved in a vehicle such as light lubricating oil. We have found the following formula to give excellent results:

125 pounds of spindle oil, 95 pounds of paraffin wax, 25 pounds of Japan wax, 1 pound of citronella and lemon oil mixed equally.

The paraffin wax and Japan wax are preferably melted and brought to a temperature of about 150 degrees and then mixed with the spindle oil which has been previously raised to about the same temperature. The ingredients are then thoroughly stirred together and may be applied to the cordage at once in the ordinary manner in which cordage oil is applied, namely, by sprinkling

the same on the fiber at the breakers. If it is not desired for immediate use it may be poured into suitable containers and allowed to cool. At normal temperatures it is a semi-solid or solid and may be stored in containers. To prepare it for use it should be gently warmed until it has melted and the mixture has come to a temperature in the neighborhood of 150 to 180 degrees 10 Fahrenheit.

Our improved cordage is made up in the usual manner of manufacturing cordage from the fibers impregnated in the manner described.

15 The vehicle employed in the compound must be a solvent for the waterproofing waxes and non-volatile at ordinary temperature and pressure. It should have the viscosity of lubricating oil, preferably light 20 lubricating oil and may consist of mineral oil such as cylinder oil, red oil, spindle oil, paraffin oil, neutral oil, petrolatum or the like or vegetable or animal oils having similar physical characteristics. It preferably does 25 not exceed 60% of the impregnating compound by volume but in any event should be sufficient to give plasticity to the particular wax or waxes employed.

30 The waterproofing waxes are preferably of two sorts, a mineral wax and a non-mineral wax.

Any mineral wax may be employed such as ceresine, ozokerite, Montan wax, lignite wax, paraffin, shale wax, or the like. Its 35 function is to penetrate the cells of the fiber and lubricate them and make them substantially waterproof. It preferably constitutes about 30% of the volume of the compound.

40 The non-mineral wax may be beeswax, carnauba wax, palmwax, wool wax, insect or China wax, Japan wax, spermaceti, stearin, or similar substances or esters having similar physical properties. It has the function of a binder to make the compound 45 more adhesive and more water repellent so that it is retained in more intimate contact with the fibers of the rope and resists abrasion. It preferably constitutes about 10% of the compound by volume.

50 In addition a small quantity of essential oil may be employed for the purpose of giving a pleasant odor to the compound and to the rope with which it is treated. Examples of such oils are mirbane, anise-rosemary, 55 citronella, sassafras, wintergreen, lemon oil, etc. The lemon oil has the additional advantages of bleaching the fiber somewhat to give it a more desirable color.

60 We are aware that petroleum oil has long been used as a lubricant for cordage and that it is commonly mixed with wool grease which has the capacity of penetrating the fiber and making it softer and smoother, but wool grease is unstable and the combination of the same with petroleum oils is emulsifi-

able in water, the emulsion being in a short time washed out by the water whereby the lubricant is driven off and the rope left subject to rapid deterioration. Furthermore the emulsion operates to release dilute fatty acids which are likely to attack the fiber and produce further emulsification of any remaining lubricant. Such rope, furthermore, becomes discolored with age so that it cannot be sold as new rope after storage. 75

We are also aware that waterproofing compounds have heretofore been suggested containing waterproofing waxes and a vehicle. But so far as we are aware no waterproofing compound for cordage has been suggested 80 prior to our invention wherein the vehicle was of such character as to permit any appreciable quantity of the waxes to penetrate the cell walls into the interior of the fiber cells. For when water or volatile hydrocarbons, 85 such as naphtha, gasoline, benzine or the like, are used as vehicles the cell walls act as filters to permit entrance only of the vehicle and to exclude the waxes from the interior of the cells so that they form a solid and relatively 90 inflexible film or deposit outside of the cells and are thus liable to wear and rub off through use. Furthermore such hydrocarbon vehicles tend to dissolve out the natural waxes contained in the cells and so leave the 95 cells with less interior protection. Such structures are doubly liable to attack by water or dampness for the wearing off of the wax film removes the waterproofing agent and the evaporation of the vehicle 100 within the fiber cells leaves room for water to enter and take its place. Cordage so treated is neither permanently water-resisting nor permanently lubricated.

105 By our invention of an impregnating compound which is capable of penetrating the cell walls so as to fill the cells with a homogeneous water-resisting compound we are able to provide a rope which is practically waterproof, which retains its flexibility, 110 lightness and ease of handling even after long immersion in water, and which is permanently lubricated. In cordage treated according to our invention, the compound in 115 the fiber cells prevents water from entering the cells, and the cell walls in turn prevent the compound from wearing or rubbing off in use. The compound being semi-solid at ordinary temperature remains permanently 120 plastic and flexible and so conforms to the changes in shape of the fiber cells in use. It results that the life of the rope and its maximum utility and strength are very materially prolonged. The compound has no 125 harmful effect upon the fiber and prevents discoloration with age. It is stable for the life of the rope structure and adds to the resistance against the action of acids on the rope. By our invention we have made rope having two to five times the durability in 130

marine use of the best lubricated rope heretofore known besides important advantages, such as continued softness, lightness and flexibility despite prolonged exposure to rain or sea water, avoidance of shrinking and kinking, avoidance of the necessity of hanging the rope out to dry, etc.

In defining our impregnating compound herein as "stable" we mean that it is of such character as to remain a homogeneous solution substantially unchanged by exposure to the elements at normal temperatures and during ordinary use of the cordage that it impregnates. By "plastic" we mean that the compound is a non-brittle substance which at normal temperatures is semi-solid and freely conforms to changes in shape of the surfaces with which it may be in contact. Our impregnating compound is both stable and plastic and, as applied to cordage, it has the capacity of passing in and out of the fiber cells so as to act both as an internal and an external lubricant of the fiber.

It will, of course, be understood that the foregoing description of our invention is illustrative only and that the invention is not intended to be limited except as defined in the appended claims.

What we claim and desire to secure by Letters Patent of the United States is:—

1. Cordage fiber the cells of which contain a stable and plastic composition consisting essentially of a waterproofing wax and a non-volatile plasticizing agent for the wax.

2. Water resisting cordage comprising fibers impregnated with a stable plastic fiber-penetrating composition consisting essentially of mineral wax and a non-volatile oil in quantity sufficient to plasticize the wax.

3. Cordage comprising fibers impregnated with a stable and plastic composition consisting essentially of mineral wax, a non-mineral wax-like substance and a non-volatile solvent in quantity sufficient to plasticize the same.

4. Permanently lubricated cordage comprising fibers the cells of which contain a plastic and stable solution of waterproofing

waxes in non-volatile mineral oil, the quantity of oil exceeding that of the waxes, said solution impregnating said fiber cells and preventing the admission of water thereto and being protected from wearing off in use by the walls of said cells.

55

5. Water resisting cellular material the cells of which contain a stable, plastic solution of mineral wax and non-mineral wax in a non-volatile vehicle, the volume of waxes being less than that of the vehicle and the vehicle being of viscosity sufficient to convey the waxes through the cell walls into the interior thereof.

60

6. Water resisting material composed of cellular fibers, the cells of the fibers containing a stable and plastic solution of a waterproofing wax in a non-volatile vehicle, the said solution containing an oil-soluble wax-like binder to cause the solution to adhere within the fiber cells, the quantity of the vehicle being sufficient to make the said solution plastic.

65

7. Water resistant cellular material the cells of which contain a stable and plastic composition of paraffine wax, an oil-soluble wax-like binder and a non-volatile oil, the quantity of oil being sufficient to render the composition plastic and capable of penetrating the said cells.

70

8. Water resistant cellular material the cells of which contain a stable and plastic composition consisting of paraffine wax, an oil-soluble wax-like binder and a non-volatile oil, the quantity of wax being greater than that of the said binder and less than that of the said oil.

75

9. Water resistant cellular material the cells of which contain a stable and plastic composition comprising approximately 30 parts of paraffine wax, approximately 10 parts of an oil-soluble wax-like binder and approximately 60 parts of non-volatile oil.

80

In testimony whereof, we have signed our names to this specification.

THOMAS T. GRAY.  
WALTER L. FAUST.  
MALVIN R. MANDELBAUM.